

May 28, 1929.

J. G. AYERS, JR

1,715,268

METHOD OF MAKING BEARINGS

Filed April 1, 1927



FIG. 1.



FIG. 2.



FIG. 4.



FIG. 5.

INVENTOR:  
JOSEPH G. AYERS, JR;  
BY *James G. Moore*,  
HIS ATTORNEY.

## UNITED STATES PATENT OFFICE.

JOSEPH G. AYERS, JR., OF MONTCLAIR, NEW JERSEY, ASSIGNOR TO GENERAL MOTORS CORPORATION, OF DETROIT, MICHIGAN, A CORPORATION OF DELAWARE.

## METHOD OF MAKING BEARINGS.

Application filed April 1, 1927. Serial No. 180,140.

This invention relates to bearings and comprises all the features of novelty herein disclosed in connection with a method of making race rings for roller bearings.

5 Hitherto, split rings or sleeves have been made from a flat strip of cold rolled steel by blanking out a piece and rolling it into the form of a ring. In order to give the ring wearing qualities suitable for modern bearings, it is hardened by heat treatment and 10 quenched. Such a piece is so apt to go out of round, even with the use of a quenching fixture and clamp to hold it, that it must be subsequently ground and this may increase 15 the cost to an extent making only a little saving over the cost of a continuous or unsplit ring, which is better.

An object of the invention, accordingly, is to provide an improved method of making 20 split race rings of a quality acceptable for use in modern roller bearings.

To these ends and to improve upon methods of the character indicated, the invention also consists in the various matters herein- 25 after described and claimed.

In the drawings, Figure 1 is a plan view of the strip material, broken lines indicating a blank to be cut from the strip.

Figure 2 is a plan view of the blank.

30 Figures 3 and 4 are side views indicating a blank being rolled into the form of a ring.

Figure 5 is a perspective view of the completed ring.

A strip 4 of cold rolled steel is first heat 35 treated and quenched in oil in the flat condition whereby distortion is avoided or minimized. A suitable heat for carbon-vanadium steel containing .55 to .65% C and .05% or more vanadium is 1550° F. The strip is 40 then too hard to roll into a sleeve so the physical properties are modified. This is satisfactorily done by packing in carbonaceous material, bringing the strip slowly to a temperature of 900 to 1100° F. and main- 45 taining the heat about one hour. This produces a homogeneous and uniform grain

structure and a smooth surface suitable for a race ring. The strip has a much more homogeneous structure than cold rolled steel and is harder but nevertheless can be rolled. 50

The blank 6 to be rolled preferably has one end 8 of V-shape and the other end 10 of corresponding shape so that, when rolled, a so-called "fish tail" joint is formed. The blank is also provided with holes 9 which become 55 oil holes in the assembled bearing. If the cut blanks are heat treated individually in the flat condition, as may be done, the holes 9 serve as a convenient means to support the blanks on pins for quenching. The pointed 60 end 8 is bent a little to facilitate the presentation of the piece to the rollers of any suitable rolling apparatus. In the illustrated apparatus, rollers 12, 14 and 16 are mounted to rotate on parallel axes, the roller 12 turning 65 clockwise and the other rollers turning counterclockwise. The piece is rolled into the form of a ring which is removed from the roller 12 by axial movement, the roller having at one end a suitably movable bearing 70 support. The rolling operation tends to iron out any distortion that may have occurred in the treatment of the flat piece. A further burnishing operation may be given, if desired, but the ring is so nearly round and so 75 smooth that grinding is unnecessary.

I claim:

The method of making a split ring with a hard raceway surface suitable for roller bearings which consists in heat treating and 80 quenching cold rolled steel in its flat condition to get a hard surface with minimum distortion, heat treating the hardened strip to produce a homogeneous and uniform grain structure, and thereafter rolling the strip to 85 iron out distortion and bend it into the form of a race ring of the required diameter for the rollers; substantially as described.

In testimony whereof I hereunto affix my signature.

JOSEPH G. AYERS, JR.